

## UNITED STATES PATENT OFFICE

2,534,178

## MANUFACTURE OF PERMANENT MAGNETS

Charles Marquaire, Ugine, France, assignor to  
 Societe D'Electro-Chimie, D'Electro-Metallurgie et des Acieries Electriques D'Ugine, Paris,  
 France, a corporation of France

No Drawing. Application February 7, 1947, Serial  
 No. 727,296. In France February 15, 1946

4-Claims. (Cl. 148—16)

1

This invention relates to the manufacture of permanent magnets through agglomerating metallic powders.

Several methods are known at present for manufacturing such magnets. Thus, in the prior applications Ser. Nos. 585,399 and 588,766, now Patent No. 2,463,413, means have been described which make it possible to obtain, by such methods, permanent magnets of a high quality.

It has been explained more particularly, in the said patent applications, that metallic powders, the particle size of which is of the same order as that of colloidal powders, should be compressed, preferably in a cold state or without letting the temperature rise higher than 250° C. and, in any case, at a sufficiently low temperature for avoiding a sintering or even a coalescence of the particles. Such a coalescence was considered as capable of modifying and decreasing the magnetic features of the finished magnet and more particularly of reducing the coercive force, it having been found that high magnetic qualities could be obtained in the magnets only by using very fine-particle powders.

However the so obtained magnets sometimes show a certain brittleness, particularly when the magnetic pieces are provided with sharp angles.

The present invention has for its object to provide a method which makes it possible to considerably improve the mechanical resistance of magnets obtained by the above mentioned methods without substantially reducing their magnetic features or even while increasing the latter. The said method consists in causing the magnet to undergo, during the agglomeration operation or after the latter, a heating in a neutral or reducing atmosphere to a temperature around 300 to 450° C.

We have discovered that, when the magnets manufactured according to the methods described and claimed in the above mentioned patent applications undergo a treatment at about 300° C. in a neutral or reducing atmosphere, their mechanical properties are considerably improved while their magnetic qualities are not substantially reduced. We have also discovered that when the temperature of the heat-treatment is increased above the latter temperature, the mechanical properties are further increased in a very substan-

tial proportion while, within a certain temperature interval, said variations are accompanied only by a very small reduction of the "quality factor" (max. BH) while a very strong increase of the remanent induction may be noted, together with a reduction of the coercive force. The practice of the method according to the present invention thus makes it possible to act upon the shape of the magnetisation curve and, accordingly, to manufacture a magnet showing the magnetic features which are the better adapted to the use for which it is designed. In opposition with what happens when massive magnets undergo heat-treatment, the importance of the variations achieved through the method according to the invention on magnets manufactured according to the above mentioned patent applications is considerable. It was thus possible to change the magnetisation curve of a magnet, similar to that of known massive magnets based on nickel-aluminum, into a curve similar to that of a massive magnet made of steel containing 35 per cent cobalt, this result being obtained by the sole heat-treatment forming the subject matter of the invention.

The following are a few examples of working out of the method described above.

*Example I*

30 A magnet was manufactured by agglomerating when cold, by compression after drowning in acetone, a powder obtained by precipitation by cooling from a mixed solution of iron and calcium formates and by decomposition of the precipitate with simultaneous reduction by heating it at 320° C. for one hour in an atmosphere of hydrogen, the flow of which was 0.1 g. per minute per gram of formate; this magnet was then heated for one hour at 315° C. in an atmosphere of wet hydrogen; the modifications of its magnetic properties were the following:

|                       | Br    | Hc  | max. BH            |
|-----------------------|-------|-----|--------------------|
| before treatment..... | 6,300 | 400 | $0.95 \times 10^6$ |
| after treatment.....  | 6,600 | 390 | $1.06 \times 10^6$ |

Mechanical resistance was multiplied by 2.6.

Shear strength of the angles was multiplied by 4.7.

Dimensions of the magnets were reduced by 1 per cent.

## Example II

A similar magnet underwent a heat-treatment at 350° C. during one hour in an atmosphere of wet hydrogen; the modifications were the following:

|                       | Br    | Hc  | max. BH           |
|-----------------------|-------|-----|-------------------|
| before treatment..... | 6,300 | 400 | $0.9 \times 10^6$ |
| after treatment.....  | 7,300 | 335 | $1.1 \times 10^6$ |

Traction strength was multiplied by 3.9.  
Shear strength of the angles was multiplied by 5.3.  
Dimensions of the magnet were reduced by 2.5 per cent.

## Example III

A similar magnet was heated during one hour at 395° C. in an atmosphere of wet hydrogen; the modifications were the following:

|                       | Br    | Hc  | max. BH            |
|-----------------------|-------|-----|--------------------|
| before treatment..... | 6,500 | 395 | $0.95 \times 10^6$ |
| after treatment.....  | 8,500 | 255 | $0.92 \times 10^6$ |

Mechanical resistance was multiplied by 4.5.  
Shear strength of the angles was multiplied by 7.  
Dimensions of the magnet were reduced by 5.5 per cent.

## Example IV

A similar magnet was heated during one hour at 450° C. in an atmosphere of wet hydrogen; the modifications were the following:

|                       | Br    | Hc  | max. BH            |
|-----------------------|-------|-----|--------------------|
| before treatment..... | 6,400 | 395 | $0.97 \times 10^6$ |
| after treatment.....  | 8,700 | 190 | $0.72 \times 10^6$ |

Mechanical resistance was multiplied by 10.5.  
Shear strength of the angles was multiplied by 18.  
Reduction of the dimensions of the magnet: 10 percent.

## Example V

A magnet was manufactured by agglomerating when cold a powder of iron-cobalt alloy comprising 33% cobalt obtained by precipitation by cooling from a mixed solution of iron and cobalt formates and decomposition of the so obtained syn-crystals with simultaneous reduction by heating at about 350° C. in an atmosphere of hydrogen. This magnet was then heated up to 360° C. in hydrogen during one hour; it underwent the following modifications:

|                       | Br    | Hc  | max. BH            | max. BH        | apparent density |
|-----------------------|-------|-----|--------------------|----------------|------------------|
|                       |       |     |                    | $Br \times Hc$ |                  |
| before treatment..... | 7,070 | 513 | $1.54 \times 10^6$ | 0.425          | 4.45             |
| after treatment.....  | 8,100 | 355 | $1.31 \times 10^6$ | 0.456          | 4.48             |

The shear strength of the angles was multiplied by 3.

## Example VI

A similar magnet was heated during one hour at 480° C. in hydrogen; it underwent the following modifications:

|                       | Br    | Hc  | max. BH             | max. BH        | apparent density |
|-----------------------|-------|-----|---------------------|----------------|------------------|
|                       |       |     |                     | $Br \times Hc$ |                  |
| before treatment..... | 5,670 | 517 | $1.12 \times 10^6$  | 0.382          | 4.28             |
| after treatment.....  | 6,850 | 347 | $0.975 \times 10^6$ | 0.410          | 4.53             |

Shear strength of the angles was multiplied by 7.5.

One considerable practical interest of the invention consists in the fact that magnets treated according to the above described method may advantageously be used in the manufacture of modern type electricity meters because of their magnetic features as well as of their mechanical properties and may be placed among the best magnets available for wide sale meters. The method makes it possible to manufacture magnets of the small air-gap type without any polar masses or field closing plates, said type being frequently used in the manufacture of meters.

What I claim is:

1. In the treatment of permanent magnets obtained by agglomerating metallic powder, the grains of which are uninsulated and have dimensions of the order of those of colloidal particles, the step consisting in heating said permanent magnets in a non-oxidizing atmosphere within the range of about 300° C.-480° C. at such temperature as increases the remanent induction, decreases the coercive force and at least maintains the product of both said factors.

2. In the treatment of permanent magnets obtained by agglomerating metallic powder, the grains of which are uninsulated and have dimensions of the order of those of colloidal particles, the step consisting in heating said permanent magnets in a reducing atmosphere within the range of about 300° C.-480° C. at such temperature as increases the remanent induction, decreases the coercive force and at least maintains the product of both said factors.

3. In the treatment of permanent magnets obtained by agglomerating metallic powder, the grains of which are uninsulated and have dimensions of the order of those of colloidal particles, the step consisting in heating said permanent magnets in a non-oxidizing atmosphere during agglomeration, said heating being within the range of about 300° C.-480° C. at such temperature as increases the remanent induction, decreases the coercive force and at least maintains the product of both said factors.

4. In the treatment of permanent magnets obtained by agglomerating metallic powder, the grains of which are uninsulated and have dimensions of the order of those of colloidal particles, the step consisting in heating said permanent magnets in a non-oxidizing atmosphere after agglomeration, said heating being within the range of about 300° C.-480° C. at such temperature as increases the remanent induction, decreases the coercive force and at least maintains the product of both said factors.

CHARLES MARQUAIRE.

## REFERENCES CITED

60 The following references are of record in the file of this patent:

## UNITED STATES PATENTS

| Number    | Name                 | Date          |
|-----------|----------------------|---------------|
| 1,669,643 | Andrews et al. ----- | May 15, 1928  |
| 1,840,352 | Elmen -----          | Jan. 12, 1932 |
| 1,859,067 | Beath -----          | May 17, 1932  |
| 2,298,885 | Hull -----           | Oct. 13, 1942 |

## FOREIGN PATENTS

| Number  | Country             | Date          |
|---------|---------------------|---------------|
| 590,392 | Great Britain ----- | July 16, 1947 |